

1,333,767.

C. NAPIER.  
METHOD OF MAKING TEMPERED BLADES.  
APPLICATION FILED DEC. 9, 1918.

Patented Mar. 16, 1920.

Fig. 1.



Fig. 2.



Fig. 3.



Fig. 4.



Inventor,  
Charles Napier,  
by Robert Bushman  
his Atty.

# UNITED STATES PATENT OFFICE.

CHARLES NAPIER, OF SPRINGFIELD, MASSACHUSETTS, ASSIGNOR TO NAPIER SAW WORKS INC., OF SPRINGFIELD, MASSACHUSETTS, A CORPORATION OF MASSACHUSETTS.

## METHOD OF MAKING TEMPERED BLADES.

1,333,767.

Specification of Letters Patent. Patented Mar. 16, 1920.

Application filed December 9, 1918. Serial No. 265,836.

*To all whom it may concern:*

Be it known that I, CHARLES NAPIER, a citizen of the United States of America, and resident of Springfield, in the county 5 of Hampden and State of Massachusetts, have invented new and useful Improvements in Methods of Making Tempered Blades, of which the following is a specification.

10 This invention relates to the heat treatment of metal articles, and concerns especially the improvement of articles dependent upon such treatment for their useful qualities, such as blades for saws, knives 15 or other cutting implements. The invention comprises an improved method or art of making a blade or tool having new and valuable characteristics.

In my Letters Patent No. 1,291,576, dated 20 April 3, 1917, I have explained a machine for uniformly tempering saw-blades, and in my Letters Patent No. 1,265,944, dated May 14, 1918, I have explained a method of heat-treating such blades adapted to be carried 25 out with the aid of such a machine, the product of the later patent being a uniformly tempered blade with annealed or soft ends useful as a hack-saw and for other purposes. Such blades are first hardened and then 30 draw-tempered throughout their middles and edges to the degree of hardness or temper heretofore customary for such blades. This customary degree of temper is such, in the instance of the hack-saw, band-saw 35 and other such blades of prior knowledge, as to provide a moderately flexible and resilient blade uniformly hard enough to enable any of its edges to serve as a metal-cutting edge, the finished blade proper, including the edge, being thus characterized 40 by a uniform crystalline structure with a low elastic limit, and therefore being brittle against sharp bending or sudden blows. In the best practice of which I am aware, I 45 have collected statistics showing that more than 42 per centum of hack-saw blades are broken in use before the usefulness of the cutting edge is impaired at all by wear. Such breakage represents a loss of value

of a still higher figure if breakages after 50 a partial use of the tool should be included.

A principal object of the present invention is to avoid such losses of value by the provision of an efficient and practical way of making a blade having a cutting edge 55 of greater hardness than has heretofore been practicable and a body which will not break under the ordinary strains of use.

Available tool-steels have heretofore necessitated for such uses a compromise between resilient flexibility and hardness, a high elastic limit being attained by draw-tempering with any available material only upon treatment resulting in reducing the hardness of the metal below an attainable, 60 and for metal-cutting purposes, the most useful value or degree. For instance, it is 65 my experience that a "glass-hard" state, attained by first heating to a high critical temperature and then chilling or quenching, is most useful for the edges, points or teeth of a metal-cutting saw, knife, or milling cutter in respect to its attack upon the material; but it is also my experience that 70 this state is impracticable for such an instrument as a saw-blade, because the desirable quality of extreme hardness is accompanied by such brittleness and susceptibility 75 to breakage in use as to limit unduly the life of the tool.

It has therefore been customary heretofore to sacrifice the quality of maximum hardness in favor of an increased springiness and toughness, the blades being tempered by subjection to a moderate uniform 80 heating after hardening so as to stand moderate bending without breakage, despite the fact that this treatment reduces the extreme hardness of the cutting edge which it would have been advantageous to retain if there 85 were any way to keep it compatible with securing toughness and resilience. When hard enough to cut, the blade still remains so brittle as to require the most careful use.

I have discovered that a cutting edge of 90 such a tool as a knife, band-saw or hack-saw blade may be kept at a point at or near its maximum hardness, thereby to pro-

duce a cutting tool of heretofore unknown durability and efficiency, if the hard edges or portions are supported by intimate and integral contact with portions of the body 5 of the blade gradually decreasing in hardness and increasing in resilience or softness within the hard points or edges. For instance, points or edge portions which have been heated above the hardening reaction 10 point, quenched or chilled, [and if desired slightly draw-tempered to an extent not reducing the desired hardness for cutting at a low heat, about 350° F. for instance, for tool-steels of usual composition] may be supported upon integral bases or a backing of 15 the same metal which has been first hardened and then drawn, as the edge is recessed from, at temperatures varying with the extent of recession from the hard points 20 or edges from about 350° to about 800° F., or such other temperature as will leave the article in a springy resilient state. Such a spring temper is a highly desirable quality of the blade proper of such an article, but 25 it is not compatible with sufficient hardness for metal cutting, and is as detrimental at the ultimate cutting edge or point as it is valuable in the body of the tool.

I do not herein claim such a blade or tool 30 as an article of manufacture, that part of my invention being the subject of a divisional application Serial No. 274,006, filed Jan. 30, 1919, for separate Letters Patent.

I have devised and will hereinafter describe a method or art of rapidly, uniformly, and if desired, continuously treating such articles so as to provide them with hard cutting points or edges and with gradually and increasingly softer and more flexibly resilient supports for the point or edge 40 within the point or edge, and with uniform spring-tempered bodies integral with and bearing such support and edge. As an article of manufacture, the resulting product 45 retains the cutting quality of hard teeth or edges against long wear, and resists breakage remarkably. I shall herein describe as an instance of the genus of new articles characterized by my invention a hack-saw 50 blade, and I shall also herein describe as one instance only of the method of heat-treating such a blade also constituting a part of my invention, steps specifically applicable to this particular article, but applicable without change except of apparatus or degree to the treatment of other specific articles included among the new genus of 55 articles comprising my invention.

In the accompanying drawings,—

60 Figure 1 is a diagram elevation of a typical specimen of the article of manufacture;

Fig. 2 is an enlarged detail of the area 2—2 of Fig. 1;

Fig. 3 is a diagram section on line 3—3 of

Fig. 2 illustrating graphically the relative 65 hardness of the metal at different parts;

Fig. 4 is a diagram plan of preferred apparatus for practising the method;

Fig. 5 is an enlarged detail diagram in plan showing relationships of temperatures 70 and previous conditions of the metal being treated; and

Fig. 6 is a detail section at the edge-heater showing one arrangement for differentially heating the parts of the articles. 75

Referring now to Figs. 1, 2 and 3, if the instrument is a saw, a preferred state of the metal is that in which the blade 10 is uniformly spring-tempered to a flexible resilience with a high elastic limit throughout the 80 region 13 comprising the greater part of the body or blade; and in which the points, faces and cutting edges 15 of the teeth are of the maximum hardness compatible with enough tensile coherence to prevent chipping or shivering. At the ultimate edges and points, this may be the maximum crystalline hardness which the metal is capable of assuming, such as will follow heating above the critical temperature [1200° to 90 1400° F. or higher for tool steels of commercial composition] and immediate quenching at temperatures at or below 350° F.

If any considerable depth of the teeth or edges of the saw is in such a crystalline 95 state, breakage under use is inevitable. For instance, if a whole tooth comprising the points and edges and faces 15 and the base or root 16 is in this state, breakage of that tooth under lateral strain or a sharp blow or 100 bending of the blade at a moderate angle is to be expected. If the region 14 adjoining the teeth is glass hard, such a breakage may involve two or more teeth. But if only the faces and edges and points are of a crystalline hardness, if the roots or bases 16 are hard but tough, and if the region 14 back of the roots 16 partakes of the qualities of resilience and flexibility, breakages of teeth do not occur. Desirably, then, the hard points and 105 faces 15 and the spring-tempered body 13 are separated by a region 14 partaking of the qualities of the hard parts at these parts, and of the quality of the springy part at the juncture at line  $\alpha$  of the blade, which may 110 be near the toothed or cutting edge. I have found that the best results for efficiency and durability are attained when the region 13 is uniformly spring-tempered and when the region 14 increases in hardness from uniformity with the temper of region 13 from the line  $\alpha$  toward the toothed edge. As shown graphically in Fig. 3, a curve  $\alpha$  whose ordinates represent hardness at abscissæ successively approaching the edge 115 rises to a maximum at the edge.

Preferably the blade is of the kind provided with perforations 11 at each end and

with soft or annealed regions 12 at the neighborhood of the perforations, responding in this respect to the product of the art or method set out in my said Letters Patent No. 1,265,944. The blade proper, comprising the regions 13 between the regions 12, 12, and the edge region 14 has first been subjected to heating above a critical temperature dependent on the material [for instance to the cherry-red hardening temperature for tool steels of usual carbon contents adapted to take a hardening reaction at the cherry-red temperature]; has been thereafter subjected to sudden cooling, as in an oil-bath; and the region 13 only has been tempered by subjection to a temperature in a neighborhood of 800° F., more or less, in accordance with the reaction of the particular metal under treatment at the hardening stage.

The region 14 and the faces, edges and points 15 have been subjected to steps first hardening these regions uniformly; then heating them above the temperature for hardening reaction; then chilling or quenching; and then "drawing the temper" of the region 14 and the bases of the teeth, points or edges by regulated causation of temperatures decreasing toward the edges or points and acting during a predetermined time only, the effect being to spring-temper the part of the strip or region 14 at its juncture with the spring-tempered blade, and to leave unaffected the condition attained at the edges or points when the edge containing them was quenched or chilled. Preferably the quenching of the edge strip 14 was so conducted as to occur at a regulated minimum temperature consonant with drawing the temper of the inner side of the strip and the inner parts of the metal blade during maintenance of this temperature at the chilled faces, edges and points.

These qualities of the product will best be understood by explanation of a specific preferred instance of the steps taken in making on a commercial scale articles of the kind referred to.

Referring now to Figs. 4, 5 and 6, the process is preferably practised continuously by subjection of a series of the articles to be treated successively during predetermined times to the different stages of treatment. A convenient way to do this is to provide for joining the articles end to end in a chain and to move them forward, for instance by such means as disclosed in my said Letters Patent No. 1,221,576, dated April 3, 1917, at a constant rate (either intermittently by short steps or continuously) past heating, quenching, reheating, tempering, cooling and washing devices suitable to the particular result desired; but it will be understood that any desired means for subjecting the

articles in succession to the described stages of treatment may be employed.

The individual articles 10 first pass through a gas-heated muffle-furnace 20 in which the articles 10 and their connectors 9 are heated uniformly. Preferably the articles, if for saws, are of steel of one of the following typical analyses:

*Carbon steel.*

|            | Percentages. |      | 75 |
|------------|--------------|------|----|
|            | Min.         | Max. |    |
| Carbon     | 1.05         | 1.10 |    |
| Manganese  | .20          | .30  | 80 |
| Sulfur     | .015         | .08  |    |
| Phosphorus | .015         | .09  |    |
| Silicon    | .035         | .045 |    |
| Nickel     | .003         | .006 |    |

*Tungsten steel.*

|            | Percentages. |      | 85 |
|------------|--------------|------|----|
|            | Min.         | Max. |    |
| Tungsten   | 1.10         | 1.25 | 90 |
| Manganese  | .20          | .30  |    |
| Sulfur     | .08          | .010 |    |
| Phosphorus | .09          | .015 |    |
| Silicon    | .010         | .015 |    |
| Carbon     | 1.10         | 1.20 |    |
| Nickel     | .00          | .003 |    |

In either case a temperature at muffle 20 of from 1350° to 1400° F. is satisfactory, and this is readily attained during progress of the saws at about 14 feet a minute through a hot passage about three feet long. 100

From the muffle the saws pass to a quenching tank 30 in which a suitable liquid, such as an oil or emulsion at about 100° F. chills the saws to a uniform glass-hard state, except at the ends, which are prevented from 105 rapid cooling by the mass of holders 9, and remain soft.

The saws now pass into a heater 40 in which the blades are heated to about 800 to 850°, to draw the temper of the region 13 to a spring temper, and to heat the edge strip 14, 15, again to a red heat at 1400° or more. Preferably a metal block 41 channeled at 42 to receive all of the saw-blades except the strip 14, 15, is positioned to receive a predetermined length of the traveling chain of saws. Heater 40 may comprise a block 41 and a refractory screen 43 supported on a base 44, and adjustable gas-blasts 45 playing downward upon the exposed edge strips 14 and the block 41. By proper regulation of the length and mass of the block 41, the intensity, temperature and number of the gas-blasts 45, no difficulty is found in maintaining the relative temperatures of the regions 13 and 14 of the saws at exit from the heater 40 at the desired figures, which are near or slightly in excess of 115 120 125

800° and 1400° F. respectively for the body and edge strip, as indicated in Fig. 3. The block 41 may be about ten inches long for an article-chain speed of 14 feet a minute. 5 Saws which were cool and glass-hard before entering heater 40 thus leave it differentially heated to degrees adapted to cool slowly to a spring temper and to chill to hardness respectively at the regions 13 and 14.

10 The heated blades are now subjected to treatment at a bath 50 adapted to resist too rapid cooling of the region 13; and first to quench or chill the strip 14 and the faces, edges and points at the edge 15, and therefore 15 after to permit the residual heat of the body 13 and strip 14 to effect a predetermined drawing of the temper of the strip 14. A preferred treatment comprises subjecting the hot running chain of blades to the action of a stream of high flash-point oil 20 from a nozzle 51 at a temperature near 350° F., the oil being so delivered as to cling to and follow the chain for a predetermined distance, representing a time during which 25 there is exchange of heat by conduction between the body 13 and the bath of hot oil, and during which the heat of the body 13 and strip 14, except the edges and points, falls to or near to the temperature of this 30 bath. The very hot strip 14, and especially the edges, faces and points 15 fall to this temperature so rapidly as to harden the cutting edges to the desired maximum degree; but the region 13 does not harden. I have 35 discovered that there is a sufficiently rapid drop of temperature at the points and edges from red heat toward the temperature of the hot oil bath to carry out this reaction; that in a bath as described at or near 350° 40 the tempering reaction at parts which have been heated only to a moderate temperature near 800° continues to the improvement of resilience and flexibility, and that a spring temper is under these conditions communicated 45 progressively from region 13 into strip 14 to a degree depending on the time the conditions remain as indicated in bath 50. I ascribe the observed phenomena to the action in bath 50 after the quenching of the 50 edge 14 of the residual heat of the greater mass of metal, *i. e.*, of the body 13 of the blades, since I find the distribution of hardness in the strip 14 to depend on the distance along the running chain [and hence on 55 the time] during which the hot stream in bath 50 is allowed to act. The depth inward from the edges and points 15 at which the metal is at maximum hardness varies inversely as this distance, so that the longer 60 the immersion and the time taken at this stage, the shallower will be the hardest parts. The times involved are relatively short, a period of about two seconds in the hot bath being sufficient for hack-saws less 65 than  $\frac{1}{2}$  inch thick.

The effect of the apparatus can be readily varied by adjusting the length of the stage 50. Conveniently this is done by providing means for reducing the temperature of the saws in such a manner as to limit the length 70 of the reaction due to bath 50. The apparatus shown provides a cold bath 60 adjustable toward and away from the nozzle 51 so as to limit the time of immersion in the hot oil to produce the desired effect. Bath 60 75 may comprise a screen 61 to stop the hot oil stream, and may contain an oil or emulsion at 100° F. or less.

Bath 60 is long enough to reduce the saws approximately to its own temperature. After passing bath 60 the saws may pass through any desired form of wash-tank containing a hot alkaline washing solution, after which the saws are separated from the chain, and packaged for sale.

While I have mentioned a chain of hacksaw blades, it will be understood that the method or art and the apparatus mentioned is applicable without change to treatment of other elongate articles to produce the 90 characteristic qualities above described. The treatment is adapted without change to band-saws, for instance, and produces for this use a band characterized by resilience adapted to long life under the repeated 95 bending to which such saws are subjected, and by a hardness at the teeth adapting the band saws to metal cutting to a degree heretofore unknown. Other articles, such as 100 knife-blades, circular saws and milling cutters included among the new genus may be treated by the described steps with suitable changes in the apparatus which will be obvious to skilled persons informed by this disclosure. I do not herein claim the apparatus mentioned which forms the subject of 105 my application Serial No. 269,598, filed January 4, 1919.

What I claim is:—

1. The art of treating hardened metallic 110 articles comprising tempering the body of the article to attain the qualities of toughness and flexibility, re-hardening an edge region only of the article, and treating the portion of said edge region adjoining the 115 body of the article to increase its flexibility and toughness.

2. The art of treating metallic blades comprising tempering the body of the blade to a spring temper, hardening an edge of the 120 blade, and draw-tempering the edge region between edge and body to a state of hardness intermediate between that of the edge and that of the body.

3. The art of treating metallic blades comprising first hardening and then drawing the temper of the body of the blade to a spring temper, then hardening an edge of the blade, and then draw-tempering the edge 125 region between edge and body to a state of 130

hardness intermediate between that of the edge and that of the body.

4. The art of treating metallic blades comprising tempering the body of the blade to a spring temper, hardening an edge of the blade, and draw-tempering the edge region between edge and body to a state of hardness exceeding that of the body and gradually varying from that of the body to that of the 10 edge, the edge remaining hard.

5. The art of treating metallic blades comprising first hardening and then drawing the temper of the body of the blade to a spring temper, then hardening an edge of 15 the blade, and then draw-tempering a portion of the edge region between edge and body to a state of hardness gradually varying from that of the body to that of the edge, the edge remaining hard.

20 6. The art of treating metallic blades comprising tempering the blade and hardening the edge region by subjection respectively to suitable different temperatures and thereafter lowering the temperatures respectively 25 of these parts sufficiently to chill the edge region while maintaining a state of tempering heat in the body.

7. The art of treating metallic blades comprising tempering the blade and hardening 30 the edge region by subjection respectively to suitable different temperatures and thereafter lowering the temperatures respectively of these parts sufficiently to chill the edge region while maintaining a state of tempering heat in the body during sufficient time 35 to affect the temper of the edge region at its juncture with the body.

8. The art of treating metallic blades comprising tempering the blade and hardening 40 the edge region by subjection respectively to suitable different temperatures and thereafter lowering the temperatures respectively of these parts sufficiently to chill the edge region while maintaining a state of tempering 45 heat in the body for a predetermined time during which the temper of the edge region is drawn progressively toward the edge, and thereafter cooling the blade to stop further changes of temper.

50 9. The art of treating metallic blades comprising hardening the blade, subjecting the body of the blade to heating to a degree sufficient to temper to a resilient and flexible state, concomitantly heating the edge region 55 of the blade to a temperature markedly higher than the body and sufficient for the hardening reaction, and then subjecting the whole blade to a bath at a temperature sufficiently low to quench or harden the edge 60 and edge-region, and sufficiently high not to quench, harden, or check the spring-tempered body.

10. The art of treating steel blades comprising hardening the blade, subjecting the body of the blade to heating to a tempera-

ture of the order of 800° F., concomitantly subjecting the edge and edge-region of the blade to heating to a temperature of the order of 1400° F., and subjecting the blades while so heated to the action of a bath at a 70 temperature of the order of 350° F.

11. The art of treating steel blades comprising hardening the blade, subjecting the body of the blade to heating to a temperature of the order of 800° F., concomitantly 75 subjecting the edge and edge-region of the blade to heating to a temperature of the order of 1400° F., and subjecting the blades while so heated to the action of a bath at a temperature of the order of 350° F. for a 80 predetermined time.

12. The art of treating steel blades comprising hardening the blade, subjecting the body of the blade to heating to a temperature of the order of 800° F., concomitantly 85 subjecting the edge and edge-region of the blade to heating to a temperature of the order of 1400° F., and subjecting the blades while so heated to the action of a bath at a temperature of the order of 350° F. for a 90 predetermined time, and at the expiry of said time lowering the temperature of the blades to stop the progressive drawing of the temper of the edge-region toward the condition of the body of the blade attained 95 during the preceding step.

13. The art of treating metallic blades comprising hardening the blade, subjecting the body of the blade to heating to a degree sufficient to temper to a resilient and flexible 100 state, concomitantly heating the edge region of the blade to a temperature markedly higher than the body and sufficient for the hardening reaction, and then subjecting the whole blade to a bath at a temperature sufficiently low to quench or harden the edge and edge-region, and sufficiently high not to quench, harden, or check the spring-tempered body, during a predetermined time, and thereafter subjecting the blade to a 110 bath at a temperature adapted to check further changes of the condition of the metal.

14. The art of treating metallic blades comprising subjecting the blades progressively during predetermined times to the 115 stages of treatment, first, heating above the temperature for hardening reaction; then quenching to harden throughout; then heating the bodies of the blades uniformly to a lesser heat adapted to draw the temper to a 120 springy state and subjecting the edge-regions of the blades to a temperature above the temperature for hardening reaction; then subjecting the blades to a hot bath at a temperature sufficiently low to harden the 125 edges and edge-region, whereby to maintain the tempering heat of the body of the blades; then subjecting the blades to a bath at a temperature checking further change in the condition of the blades. 130

15. The steps in the art of treating metallic articles by heat comprising heating a part of the article to the temperature for hardening reaction; concomitantly heating 5 another part of the article to a lesser degree appropriate to a tough and flexible temper, and subjecting the article while in said state of locally different temperatures for a predetermined time to a bath heated to a point 10 adapted to conserve the temperature of the cooler parts of the article and quench or chill to harden the hotter parts, whereby the temper of the hardened parts is progressively changed at and from the juncture of 15 said hardened parts with the parts heated to the lesser degree during maintenance in said bath.

16. In a method of heat-treating saw-blades, the steps comprising hardening the 20 blades, then subjecting the edge-region containing the teeth and the body of the blade of the saw respectively to local heating to a high temperature for hardening and a lower temperature for spring-tempering, quenching 25 the blades in a bath at a temperature of the order of 350°, whereby to harden the faces, points and edges of the teeth and the edge-region; and then maintaining the blades in said bath for a predetermined 30 time during which the temper of the hardened edge-region is progressively drawn by exposure to heat conducted from the body of the blade, and then subjecting the blades to rapid cooling before the temper of the 35 hardened faces, points and edges is affected.

17. The art of treating metallic blades

comprising moving the blades at a predetermined rate respectively through means for locally heating the blades to different predetermined temperatures and through a predetermined extent of a heated bath adapted to quench the hotter parts, and to permit the cooler parts to remain at a heat reacting during the time of passage in said bath to draw the temper of adjoining parts hardened when quenched to a degree determined by the extent of said bath, and the rate of motion of the blade.

40

45

18. In a method of treating metallic blades, the steps locally heating a blade running at a predetermined rate to different degrees of heat, and immediately subjecting the heated running blade to the action of a bath adapted substantially to conserve the previously attained temperature of one part 55 of the metal and to affect the hardness or temper of the metal differently at another previously heated part, the time elapsing between said steps being insufficient substantially to change the distribution of the heat 60 in the blade.

19. The method of heat-treating metallic blades comprising locally heating a blade moving at a predetermined rate to predetermined different temperatures and then subjecting the locally heated blade to the action 65 of a stream of a hot quenching agent following the blade for a predetermined distance of travel at said rate.

Signed by me at Springfield, Massachusetts, this 5th day of December, 1918.

CHARLES NAPIER.

50

55

60

65

70